

1

2,805,186

**METHOD OF PREPARING ANIMAL GLUE**

Havard L. Keil, Clarendon Hills, Louis A. Harriman, Chicago, and Arlan G. Roberts, Dolton, Ill., assignors to Armour and Company, Chicago, Ill., a corporation of Illinois

No Drawing. Application February 26, 1953,  
Serial No. 339,166

10 Claims. (Cl. 195—6)

This invention relates to a method of preparing animal glue. The method of this invention can be employed with particular advantage in preparing hide glue from cattle hide glue stock.

This application is a continuation-in-part of our co-pending application United States Serial No. 243,378, filed August 23, 1951.

The present commercial practice for preparing cattle hide glue involves the following principal steps:

1. The cattle hide glue stock is soaked in a saturated lime solution for a period of from 60 to 120 days, depending on the temperature, for the purpose of softening and conditioning the glue stock.

2. The conditioned glue stock is then soaked in water at an acidic pH to remove lime and calcium salts including the carbonates.

3. The glue stock is then washed back to approximately a neutral pH value, or neutralized with an alkaline reagent.

4. The conditioned, swollen and neutralized glue stock is then extracted with hot water in a series of "cooks" at increasing temperatures to obtain the glue.

The reason for this lengthy conditioning process is found in the fact that it is very difficult to prepare glue from hide glue stock having a high gel strength and a correspondingly high viscosity. By way of contrast, gelatin is easy to prepare. Although gelatin is almost chemically identical with glue, it has such a low viscosity that it has not been acceptable to the trade for adhesive purposes.

An isolated collagen fiber can be easily extracted to obtain glue, but when the collagen fibers are in their natural state within solid pieces of hide stock, it is very difficult to extract the glue. The pieces of hide stock must be opened up or conditioned to make the extraction feasible. A long standing problem in the field is how to do this conditioning rapidly without damaging the collagen. The conversion of collagen to glue involves a very slight change, and there is even a dispute as to whether the change can be properly described as a chemical change. It is known that the conversion of collagen to glue does not involve proteolysis in the ordinary sense, i. e., splitting of polypeptide chains.

It has been suggested that the lengthy lime conditioning process might be avoided by employing enzymes to condition the glue stock. However, the use of enzymes for this purpose has not proven practical because they degrade the collagen past the glue stage. Therefore, although there is a manifest need for a shorter process involving less handling of the glue stock, and less chemicals, no process has heretofore been developed which is capable of producing glue of a quality comparable to the high grade glues of commerce.

It is therefore a general object of this invention to provide a new process for preparing animal glue which substantially overcomes the above problems, and makes possible the preparation of high grade animal glue in a greatly

2

reduced period of time, and also requires less handling of the glue stock, and less chemicals. It is a further object of this invention to provide a novel process for preparing glue from cattle hide glue stock which achieves the broad object just stated, and at the same time produces high yields or excellent quality glue from the standpoint of gel strength and viscosity. Further objects and advantages will appear as the specification proceeds.

This invention is based in part on the accidental discovery that collagen-bearing animal tissues can be rapidly conditioned for glue extraction by subjecting the tissues to the enzymatic action of yeasts and yeast-like microorganisms.

Any collagen-bearing animal tissue can be employed as the starting material in the process of this invention. However, the process realizes its greatest advantage in the preparation of hide glue, and therefore hide glue stock, and particularly cattle hide glue stock, is preferably employed as the starting material. Cattle hide glue stock is of two principal types. It is salt-cured stock or fresh stock. The salt-cured stock is the trimmings from salt-cured hides. Fresh stock is mainly the trimmings from fresh hides, and in particular the so-called "ears" and "lips." The principal source of raw material is salt-cured hide trimmings. Hides from freshly slaughtered animals are cured preparatory to the tanning operation by storing in cellars for a period from 30 to 60 days. The hide cellars are maintained at a temperature of about 10° C. and the hides are stacked in piles with a layer of rock salt between the individual hides. When the curing is complete the hides are trimmed, bundled and shipped to the tannery. The scrap pieces trimmed from the cured hides are then utilized as the raw material for the manufacture of hide glue.

In practicing the process of this invention, the conditioning of the solid pieces of collagen-bearing tissue is accomplished by suspending the tissue in an aqueous acidic medium and culturing yeasts or yeast-like organisms in the medium which have a conditioning action on the glue stock. It will be understood, of course, that the aqueous medium should be maintained under pH conditions, temperature conditions, etc., which are known to be favorable to the growth of yeast and yeast-like microorganisms. The particular "yeasts" which have

been found most desirable for this purpose are the so-called "wild yeasts" of the genus *Mycoderma*. As a member of the class *Fungi Imperfecti*, *Mycoderma* belongs to the family *Torulopsidaceae*, which contains other yeast-like genera exhibiting a hide-conditioning action, such as the genus *Torulopsis*. Although *Mycoderma* organisms can be used separately, it is preferred to employ both *Mycoderma* and *Torulopsis* organisms. Apparently a synergistic relation exists between these yeast-like organisms in conditioning hide for glue extraction. In particular, the organism *Mycoderma* (*sp.*) is believed to soften the keratin layer of the hide as well as the elastin sheathes around the collagen fibers by its ability to remove sulphur from cystine, and by so doing an important cross linkage between peptide chains is broken so that the structure is weakened and at the same time is opened up so that water may enter. *Torulopsis* (*sp.*) is believed to aid in the conditioning of the hides by its ability to hydrolyze the fatty tissue present in the hide pieces, thus permitting easier penetration of the glue extraction waters to the inner hide structure.

Both *Mycoderma* and *Torulopsis* are ubiquitous organisms, being found in the air, dust, etc. These organisms are also found in quantity on cattle hides. Advantage can be taken of this fact by using the indigenous yeast organisms on the hides to inoculate the conditioning medium. This method of procedure is especially good

for salt-cured hide trimmings, since the hide cellars provide excellent conditions for the multiplication of both *Mycoderma* and *Torulopsis*, and these organisms are always found to be present in hide cellars. If desired, the aqueous medium can be inoculated with *Mycoderma* and *Torulopsis* organisms, which can be cultured for this purpose, and charged to the conditioning bath in the form of an active broth. A convenient source of these yeast-like organisms is in the so-called "hairballs," which are found in quantity at stockyards. (Hairballs are matted balls of hair and manure which are cut off the outer portion of cattle hides.)

Other organisms can also be present in the conditioning bath, and some have been found to exhibit a synergistic or at least symbiotic effect. In particular, the true yeasts of the tribe *Saccharomycetaceae*, such as *Saccharomyces*, have been found to be advantageous for this purpose. The genus *Saccharomyces* contains most of the well-known commercial yeasts, such as baker's yeast, brewer's yeast, etc., and contains such specific yeast organisms as *S. cerevisiae* and *S. carlsbergensis*. These yeasts apparently stimulate the growth of *Mycoderma* and *Torulopsis* yeasts, thereby accelerating the hide conditioning.

It is desired to maintain the aqueous conditioning medium substantially free of putrificative bacteria and molds. This can be accomplished in a number of ways. For example, the glue stock can be sterilized with a germicidal agent before it is introduced into the conditioning bath, and precautions can be taken to prevent bacteria and molds from being introduced into the bath. One sterilizing agent which might be employed for this purpose with particular advantage is hydrogen peroxide, since it can be readily destroyed by the use of catalase after the sterilization has been achieved. Alternatively, the aqueous conditioning medium can be maintained at a pH sufficiently low to inhibit the growth of bacteria and molds while permitting the growth of the desired yeasts or yeast-like organisms. This technique is described in co pending application United States Serial No. 243,378, cited above.

While the above methods of culturing yeasts and yeast-like organisms and maintaining the medium substantially free of putrificative bacteria and molds are entirely feasible, it is preferred to employ still another method of accomplishing this result in which a selective bactericide is incorporated in the conditioning medium. It has been discovered that water-soluble silicofluoride salts are particularly good for this purpose under the conditions of the process. Sodium, potassium, or ammonium silicofluorides are preferred, but other water-soluble silicofluoride salts can be used, and in particular the alkali metal silicofluorides. These salts can be used up to the limit of their solubility, but with more soluble salts such as sodium silicofluoride, it is preferred to operate with aqueous solutions at about one-half saturation. For example, a .3% aqueous solution of sodium silicofluoride is about one-half saturation.

The use of selective bactericides and particularly of silicofluoride salts permits the conditioning to be carried out at higher temperatures and pH's, thereby accelerating the growth of the desired organisms and shortening the conditioning time. In general, the conditioning step can be satisfactorily carried out at temperatures from 15 to 45° C., and best results are achieved at temperatures ranging from 20 to 40° C. When carrying out the conditioning in the presence of a silicofluoride salt, the pH should be maintained between 3.5 and 6.5 and preferably between 4.0 and 5.0. At pH's below 3.5, the silicofluoride salts have a tendency to inhibit the growth of the yeast as well as the bacteria and molds.

During the conditioning step, the pH will tend to vary somewhat, and therefore it is preferred to make periodic adjustments of the pH to maintain it within the specified limits. In making the initial and subsequent pH adjust-

ments, various organic and inorganic acids can be employed, such as acetic, nitric, phosphoric, and sulfuric, etc. Of course, it will be understood that the acid employed must not be toxic to the desired organisms. Hydrochloric acid is the reagent of preference.

The time required to complete the conditioning will vary somewhat depending on the particular conditions. It may take from 1 to 21 days to complete the conditioning, although in the preferred process as described herein usually 2 to 3 days are sufficient. The point at which the hide stock has become sufficiently conditioned can be easily determined by visual observation and by simple tests. When the hide is conditioned, it is usually quite soft and can be cut with a fingernail. Both hair and scurf (the outer epidermal layer) can be easily pulled.

The organism-conditioned glue stock can be directly extracted, after neutralization of the acid, with hot water in accordance with conventional practice. However, it is preferable to first plump or swell the glue stock by treating it in an acid bath at a lower pH than in the organism conditioning. For this swelling step, pH's of from 1.5 to 3.5 give good results, and maximum swelling is achieved at pH's ranging from 2 to 2.5. Hydrochloric acid is preferred as the acidic reagent, although many other acids can be satisfactorily employed, e. g., acetic, nitric, phosphoric, sulfuric, etc.

The temperature in the swelling step is not especially critical, and room temperatures are quite satisfactory (20 to 25° C.). A suitable range temperature for the swelling operation is from 15 to 40° C. In the swelling operation, the water penetrates the solid pieces of hide in as short a time as 3 hours, and maximum swelling may be achieved in 24 hours. There is some advantage in a longer time of contact of the glue stock with the swelling solution, and therefore it may be desirable to soak the glue stock in the acidified water for periods up to 3 to 4 days. In this way, swelling of from 210 to 225% can be achieved, as compared with swelling of from 150 to 170% in the conventional liming and plumping procedures.

The plumped stock can be washed to remove the acid contained therein, and thus brought to a neutral pH, or it can be neutralized with various alkaline reagents such as ammonium hydroxide, sodium hydroxide, sodium carbonate, etc. After neutralization, the glue stock can be extracted with hot water according to conventional procedures.

The temperatures, cooking times, and ratio of water to solids can all be satisfactorily determined according to the usual practice. For example, the glue stock solids can be covered with water and cooked for 3 hours at 65° C. to obtain a glue liquor, which can be subsequently dried or evaporated to obtain the solid glue. The glue stock residue from the first extraction can then be re-extracted once at 65° C. and then carried through a series of similar extractions at progressively higher temperatures, e. g., at 75° C., at 85° C., and 100° C.

This invention is illustrated in a number of different specific embodiments in the following examples.

#### Example I

High quality glue can be prepared from collagen-bearing animal tissue according to the following procedure:

The hide trimmings, or other collagen-bearing glue stock, is covered with water and a culture containing *Mycoderma* and *Torulopsis* is added. The water is half-saturated with sodium silicofluoride (0.3%) and sufficient hydrochloric acid is added daily to maintain a pH of 4.0-4.5. A temperature of around 35° C. is used to augment microorganism growth. After about 3 days, the hair slips readily along with the epidermal layer. The hide is then removed; and after being rinsed in running water, it is ready to go into the next step.

The rinsed stock is covered with water and hydrochloric acid added to about pH 2.0. It is held at room tempera-

ture and more hydrochloric acid added daily to maintain a pH between 2.0-2.5. At the end of 2-4 days, the hide is satisfactorily conditioned for glue extraction.

It is possible to use the first step alone. This saves much time and work since the tissue does not receive acid plumping. However, the glue thus obtained is usually of somewhat lower viscosity.

*Example II*

Thirteen pounds of fresh cattle hide trimmings were put into 4 gallons of water containing 42 grams of sodium silicofluoride. A culture of the conditioning microorganisms was added and the mixture held at 35° C. Sufficient hydrochloric acid was added daily to maintain the pH at about 4.0-4.5. At the end of 4 days, the tissue was washed in cold water for a few hours and was then subjected to the regular procedure for the extraction of glue, after neutralization.

Glue extraction consists of covering the stock with water and heating it at 65°, 75°, 85°, 95°, and 100° C. for 3 hours respectively. The glue liquors thus obtained are separately concentrated in vacuo and subsequently dried in a wind tunnel.

*Example III*

Twelve pounds of salted cattle hide scrap were washed in running water overnight to remove salt. The scrap was then put into 4 gallons of water containing 42 grams of sodium silicofluoride. A culture of the conditioning microorganisms was added and the mixture held at 35° C. Sufficient hydrochloric acid was added daily to maintain the pH at about 4.0-4.5. At the end of 3 days, the tissue was washed in cold water for a few hours, after which it was transferred to the second step.

The stock was covered with water and 50 cc. of concentrated hydrochloric acid added at 10 A. M. to pH 2.1. At 2:15 P. M. the same day the pH read 2.5, so 35 cc. of the acid was added to pH 2.0. On the following day, the pH was 2.4 at 9 A. M. 50 cc. of the acid was added to reach pH 2.0. On the next (third) day the pH was 2.2 and on the fourth day the same. An equilibrium had thus been attained on the third day of acid treatment, which shows that swelling was at the maximum.

The stock was thoroughly conditioned, so it was neutralized by water-washing for two days and the glue extracted in the same manner as that described in Example II.

*Example IV*

A 45# lot of salted cattle-hide pieces, obtained from the trimmings pile of the hide cellar, was washed for 4 hours in cold running water in order to clean, soften, and partly desalt the material. A tumbler-type washing machine was employed. A one-hour wash has been found to be sufficient to remove dirt and blood from fresh hide pieces.

The washed hides were then transferred to a 30-gal. barrel and 225 g. of sodium silicofluoride, equal to 1.11% of the as-received weight of the hide pieces, was added and the barrel filled with warm water. The pH of the mixture was adjusted to 4.0 by addition of hydrochloric acid. Barrel temperature was conveniently maintained at 35-37° C. by use of a Fenwal Thermoswitch, knife-type immersion heater, and electric stirrer to insure circulation. During the three days of this treatment, hydrochloric acid was added intermittently in order to maintain pH at 4.0. A total of 95 cc. of concentrated hydrochloric acid was employed. Lots as large as 80# have been successfully handled in this same equipment.

Treatment at pH 4.0 in the presence of sodium silicofluoride is necessary in order to obtain hair loosening and keratin softening. At the end of the first day of this treatment, hair could be pulled from many of the pieces, and by the conclusion of the third day, much loose hair was floating in the mixture.

After treatment at pH 4.0 for 3 days, the water was changed and stirring and heating were discontinued. The pH was adjusted to 2.0 by addition of hydrochloric acid and was maintained at this value for 4 days by intermittent addition of fresh acid. For the 4-day period, a total of 450 cc. of concentrated hydrochloric acid was utilized. During this 4-day period a marked change took place in the appearance of the hide pieces. Swelling in thickness and area was pronounced and occasional blistering of the hair-side keratin layer was noted. The keratin layer could easily be cut by the fingernail. Considerably more hair loosening also was evident.

Prior to actual glue extraction, the hide pieces were washed for one hour in cold running water in the tumbler-mill. This wash removed almost all the remaining hair and freed the hide surface of excess acidity, thereby diminishing the ash content of the final glue. By placing a filter screen in the effluent wash stream it is possible to collect the freed cattle hair. The hair is light in color, in good condition, and may have a useful market.

The washed hides were stored before actual glue cooking in hydrochloric acid solution at pH 2.0. Storage for extended periods has no apparent effect on glue quality since equilibrium is attained within the 4-day treatment and no additional hydrochloric acid is absorbed. The conditioned glue stock was then extracted. A schedule of four 3-hour cooks was employed. Cooking temperatures were 65°, 75°, 85°, and boiling.

Hide pieces were placed in a pot and the temperature was quickly elevated by addition of sufficient water at the desired cooking temperature to cover the hide pieces. The cooking pot was maintained at cook temperature by external heating for a 3-hour period. At the completion of the cook, glue liquors were drained, preservative (Dowicide G) was added, the solution was concentrated under vacuum, jellied, and dried either in a heated wind oven or a vacuum oven. A light-colored and frequently transparent dried glue was obtained. At the end of the fourth cook, the residue, which still appeared to contain some potential glue-forming material, was dried for weighing in the wind oven.

In a series of replicate runs following the specific procedure set out above, the average yield of glue was around 20% on an as-received basis. The average jell strength of the glue was around 440 grams, and the average viscosity was 150 millipoises.

*Example V*

Ten pounds of trimmings from salt-cured cattle hides were washed in running water for 24 hours to remove the salt and dirt. The washed hide pieces were covered with 5 gallons of water and 50 ml. of concentrated hydrochloric acid was added. The pH after the addition of the acid was 2.3. Periodically the pH was determined and sufficient acid added to maintain the pH between 2.0 and 2.5. After 5 days the surface of the bath was covered with a wrinkled gray film and the hide hair slipped easily. After the 21st day of conditioning the hide was removed from the bath and weighed up at 7304 grams. The pieces were covered with water and 3% or 219 ml. of concentrated ammonium hydroxide was stirred into the lot. The stock remained in the ammonium hydroxide solution for 24 hours and was then removed for glue cooking operations.

Glue extractions were made at 150° to 160° F., 165° to 175° F., 180° to 190° F., and 212° F. and 212° F. Fresh extraction waters were used for each heating and the temperature was maintained at each temperature range for 3 hours. The glue liquors from each cooking were removed from the stock, centrifuged, jelled and dried.

The yield of glue was 21.6% on an as-received basis. The average jell strength of the glue was 316 grams and the average viscosity 142 millipoises.

*Example VI*

Thirty pounds of salted hide scraps were washed in running water for 24 hours to remove the salt and dirt. The washed hide scraps were covered with 15 gallons of water and 150 ml. of concentrated hydrochloric acid was added. The pH after the addition of acid was 2.0. Additional acid was added as necessary to maintain the pH between 2.0 and 2.5. After 26 days some of the hide pieces were removed from the bath and weighed up at 11,579 grams. These pieces were then covered with water and 3% or 350 ml. of ammonium hydroxide was stirred into the lot. After 24 hours the stock was removed and glue extractions were made following the procedure of Example V. The yield of glue was calculated as 24.9% based on an as-received basis. The average jell strength was 317 grams and the average viscosity 135 millipoises.

*Example VII*

The remaining portion of the hide pieces from Example VI were allowed to remain in the conditioning bath for a total of 68 days. Following the conditioning operation the stock was cooked for glue extraction. The glue obtained was of high quality and the viscosity values were not adversely affected by the prolonged conditioning treatment.

*Example VIII*

One hundred pounds of salted cattle hide scrap was washed in running water for 24 hours to remove salt and dirt. The washed skins were covered with water and sufficient hydrochloric acid added to maintain a pH of 2.5. One pound of baker's yeast was added and the lot allowed to stand for 14 days at room temperature.

At the end of this time the stock was thoroughly conditioned as evidenced by a weak epidermal layer which could be cut by the thumb nail. The stock was next rinsed and weighed. This weight, due to water imbibition, was 225 pounds which denotes a 125% weight increase. The lot was covered with water and 3% or 6.75 pounds of ammonium hydroxide was added and allowed to stand for 18 hours to neutralize. Glue was extracted by the usual procedure.

While in the foregoing specification this invention has been described in considerable detail and a number of specific embodiments have been set forth, it will be apparent to those skilled in the art that many of the specific details and embodiments can be varied widely without departing from the broad idea of the invention.

We claim:

1. In a method of preparing animal glue, the steps of subjecting collagen-bearing animal tissue to reproducing yeast microorganisms of the genus *Mycoderma* indigenous to cattle hides, while maintaining said animal tissue substantially free from putrefactive bacteria and molds, and thereafter extracting glue from said collagen-bearing tissue.
2. In a method of preparing animal glue, the steps of conditioning collagen-bearing animal tissue, in an aqueous acidic medium with the enzymatic conditioning action of yeast microorganisms both of the genus *Mycoderma* and the genus *Torulopsis* indigenous to cattle hides, under conditions favorable to the multiplication of said yeast organisms while maintaining said aqueous acidic medium substantially free from putrefactive bacteria and molds, and thereafter extracting glue from the conditioned animal tissue.
3. The method of claim 2 in which said collagen-bearing animal tissue is cattle hide glue stock.
4. The method of claim 2 in which said collagen-bearing animal tissue is salt-cured cattle hide trimmings.
5. In a method of preparing animal glue, steps of conditioning collagen-bearing animal tissues in an aqueous

acidic medium with viable yeast microorganisms both of the genus *Mycoderma* and the genus *Torulopsis* indigenous to cattle hides and a yeast microorganism of the group consisting of *Saccharomyces cerevesiae* and *Saccharomyces carlsbergensis*, under conditions favorable to the multiplication of said yeast microorganisms while maintaining said aqueous acidic medium substantially free from putrefactive bacteria and molds, and thereafter subjecting the conditioned tissue to a hot water extraction to obtain the glue.

6. In a method of preparing animal glue, the steps of conditioning in an aqueous acidic medium salt-cured cattle hide trimmings, having disposed thereon viable yeast organisms of the genus *Mycoderma* indigenous to cattle hides, under conditions favorable to the multiplication of said yeast organisms while maintaining said aqueous acidic medium substantially free from putrefactive bacteria and molds, and thereafter extracting glue from the conditioned hide trimmings.

7. In a method of preparing animal glue, the steps of conditioning collagen-bearing animal tissue in an aqueous medium having a pH of from 3.5 to 6.5 with yeast microorganisms of the genus *Mycoderma* indigenous to cattle hides, under conditions favorable to the multiplication of said yeast organisms, while contacting said aqueous medium with a water-soluble silicofluoride salt to maintain said medium substantially free from putrefactive bacteria and molds, and thereafter extracting glue from the conditioned animal tissue.

8. In a method of preparing animal glue, the steps of conditioning collagen-bearing animal tissue in an aqueous medium having a pH of from 4.0 to 5.0 at a temperature of from 15 to 45° C. with yeast organisms both of the genus *Mycoderma* and the genus *Torulopsis* indigenous to cattle hides, under conditions favorable to the multiplication of said yeast organisms, while contacting said aqueous medium with a water-soluble silicofluoride salt to maintain said medium substantially free from putrefactive bacteria and molds, and thereafter extracting glue from the conditioned animal tissue.

9. The method of claim 8 in which said water-soluble silicofluoride salt is selected from the group consisting of alkali metal silicofluorides and ammonium silicofluoride.

10. In a method of preparing animal glue, the steps of conditioning salt-cured cattle hide trimmings in an aqueous acidic medium having a pH of at least 3.5 with yeast organisms both of the genus *Mycoderma* and the genus *Torulopsis* indigenous to cattle hides, under conditions favorable to the multiplication of said yeast organisms while maintaining said aqueous acidic medium substantially free from putrefactive bacteria and molds, then soaking the conditioned hide trimmings in water acidified to a pH of from 1.5 to 3.5 to swell said hide trimmings, and thereafter extracting glue from the conditioned, acid-swollen hide trimmings.

## References Cited in the file of this patent

## UNITED STATES PATENTS

- |    |           |               |                 |
|----|-----------|---------------|-----------------|
| 60 | 1,405,741 | Rohm          | Feb. 7, 1922    |
|    | 2,515,055 | Rohm          | Sept. 17, 1940  |
|    |           |               | FOREIGN PATENTS |
|    | 2,879     | Great Britain | of 1917         |
| 65 | 104,181   | Great Britain | 1917            |

## OTHER REFERENCES

- Smyth et al.: Industrial Microbiology, 1930, Williams and Wilkins, Balt., Md., pages 125-126.
- Sumner et al.: The Enzymes, Academic Press Inc. Pub., New York, 1952, pages 1317-1318.
- Lodder: The Yeasts, Interscience Pub. Inc., New York, pages 699, 700, 708 to 710.